

Sept. 24, 1929.

R. B. DANIELS

1,729,571

METHOD OF MAKING PAPER

Filed Oct. 15, 1926

2 Sheets-Sheet 1

*Fig. 1.*



*Fig. 2.*



*Fig. 3.*



Sept. 24, 1929.

R. B. DANIELS

1,729,571

METHOD OF MAKING PAPER

Filed Oct. 15, 1926

2 Sheets-Sheet 2

*Fig. 4.*



*Fig. 5.*



Inventor  
Rupert B. Daniels.

By his Attorneys  
Eugene Booth, James M. Tracy

## UNITED STATES PATENT OFFICE

RUPERT B. DANIELS, OF ADAMS, MASSACHUSETTS, ASSIGNOR TO L. L. BROWN PAPER COMPANY, OF ADAMS, MASSACHUSETTS, A CORPORATION OF MASSACHUSETTS

## METHOD OF MAKING PAPER

Application filed October 15, 1926. Serial No. 141,785.

This invention relates to the art of paper making and pertains more particularly to the making of paper having certain definite portions of a thickness different from that of other definite portions thereof.

It is an object of this invention to provide a method and apparatus which shall produce such paper expeditiously and efficiently.

Other objects and advantages of the invention will appear hereinafter.

The accompanying drawings illustrate the invention more or less semi-diagrammatically, Figure 1 being a plan view, Figure 2 being a side elevation, certain parts being shown in section to better illustrate the invention, Figure 3 is a detail perspective view, Figure 4 is an enlarged detail view, partly broken away, and Figure 5 is a section on the line 5—5 of Figure 4.

For purposes of convenience of description the invention has been illustrated as applied to the ordinary Fourdrinier paper making machine in which the stock comprising fibrous material and water is flowed in a liquid state onto a moving wire through which the water is permitted to percolate gradually, leaving the fibrous mass forming the web. In such machines the wire is caused to travel continuously at a uniform rate and the flow of stock onto the wire is ordinarily controlled by slices or bars extending across the path of the wire, said slices being arranged to permit a substantially uniform rate of flow of stock thereunder so that the web or paper which is formed may be of uniform thickness.

In my former Patents Nos. 1,587,700 and 1,587,699 I have described a method of forming a web of the type in which the fibrous mass constituting certain defined portions is of a different thickness from that constituting other portions thereof, by depositing the stock or pulp to form the web in a layer having different thicknesses at the desired different portions thereof. It was proposed in said patents to control the flow of stock past the usual slices in such manner as to provide one rate of flow at certain points and to provide a different rate of flow at other points, the web formed by so controlling the

flow of the stock having defined portions of different thicknesses. It was also proposed to maintain the difference in thickness of the pulpy mass thus established until sufficient water had been removed therefrom so that there was no further tendency for the pulp to flow from one portion to another by applying fluid pressure to the areas of less thickness sufficient to prevent the flow of pulp from one area to another.

In the specific embodiment of the invention illustrated in the drawings of the said patents the depositing of fibers on the wire was controlled at the slice by securing thereto an obstruction in the form of a U-shaped plate which restricted the flow of fibers thereunder at that point. Thereafter the areas of less thickness thus formed were maintained by applying air pressure, either in the form of a series of direct jets as disclosed in Patent No. 1,587,700 or in the form of a confined current of air as by providing a hood as disclosed in Patent No. 1,587,699.

It has been found, however, that for certain purposes, the desired restriction of the flow of stock under the slice may be secured without the use of a mechanical obstruction attached to the slice, if the air pressure which is used to maintain the areas of less thickness is applied in a manner to permit it to restrict somewhat the inflow of pulp under the slice at the point at which the air pressure is applied.

Referring to the drawings, liquid stock from the flow box 1 passes from the flow box over the lip 2 and over the apron 3 onto the wire 4 which passes about the breast roll 4' in the usual manner. As the stock flows along in the direction of the arrows it passes under the first slice 5 which is adjusted with respect to the wire 4 in such manner as to restrict the flow of stock somewhat before passing to the second slice 6. The second slice is arranged somewhat nearer the wire 4 than the first slice and ordinarily permits the flow of stock thereunder to form a layer of pulp 7 of uniform thickness. Adjacent the slice 6 and extending longitudinally along the wire is arranged the pipe 11 having a series of openings arranged longitudinally along the under

side thereof. Beneath the openings and also extending longitudinally along the under side of the pipe 11 is a baffle plate 13 which serves to deflect the incoming air current to prevent the direct application thereof to the moist pulp in order to prevent disturbance of the fibers.

On both sides of the pipe 11 and extending longitudinally thereof throughout substantially its entire length are side walls or curtains 14 comprising in the present embodiment flat metal plates secured to the sides of the pipe in any suitable manner. The pipe 11 is connected to a header 15 through the flexible hose 16 and the header may be connected to a suitable blower or other source of air pressure through the pipe 15.

Any suitable number of pipes 11 may be used depending upon the areas which it may be desirable to form in the sheet. One of the pipes 11 for the application of fluid pressure is provided, of course, for each portion of less thickness.

Each of the pipes 11 may be conveniently supported by the usual cross rods 17 for the deckle frames and may be attached thereto by any suitable means. In the present embodiment means are provided by which the pipes may be adjusted vertically with respect to the cross rods and the wire in order that the pipes may be conveniently brought into proper relationship with the web which is in the process of formation. Such means may comprise simply threaded bolts 18 passing through the straps supporting the pipes, which bolts may be turned to raise or lower the pipes as desired.

As will be apparent, the pipes 11 with their attached fins or curtains 14 form an elongated hood through which air pressure may be applied to the web. Preferably the pipe is so adjusted with respect to the wire and pulp thereof that the curtains 14 project slightly into the pulp to form a seal to prevent the escape of air along the sides thereof. The curtains 14 should not project too deeply into the pulp for best results, as it has been observed that when this occurs the fibers are sometimes disturbed by a rolling action which takes place between the lower edge of the curtains and the wire which causes undesirable effects in the finished paper.

The forward end of each of the pipes 11 is arranged closely adjacent to the second slice 56 6 and the confined body of air therein restricts the flow of pulp under the slice in such manner that less fibers are deposited at these points. By extending the hoods in the manner illustrated for considerable distance beyond the second slice 6 and thus maintaining air pressure on the thinned portion thus formed, the inflow of fibers from the areas of greater thickness is prevented until at the ends of the hoods, sufficient water 65 has been removed from the pulpy material so

that there is no further tendency for the fibers to flow from one area to another.

The adjustment of the air pressure applied is a matter of some importance, but due to the varying conditions encountered in manufacturing processes no satisfactory rule as to its amount can be given. Different rates of flow of the stock, different qualities of stock and even different atmospheric conditions may operate to vary the air pressure required.

The proper pressure may easily be determined by a skillful operator by observance of the apparatus in operation, for the pressure applied should in no case be sufficient to cause the pulp to be extruded beneath the fins or curtains 14. In fact, in order to avoid this result with the accompanying undesirable ridge which would be formed thereby on either side of the portion of less thickness, it is preferable to reduce the air pressure to a point where some inflow of pulp may result, as this has no ill effect on the finished paper, although it will be understood that the ideal condition is that in which no flow occurs in either direction.

It will be understood that the invention may be variously modified and embodied within the scope of the subjoined claims.

I claim as my invention:

1. The method of controlling the flow of fibers to form a paper sheet having designated areas of less thickness than the normal thickness of said sheet, which comprises restricting the flow of fibers to the areas of less thickness to a greater extent than to the areas of normal thickness by applying fluid pressure, and maintaining the difference in thickness until the fibers are set by continued application of fluid pressure.

2. The method of controlling the flow of fibers to form a paper sheet having designated areas of less thickness than the normal thickness of said sheet, which comprises restricting the flow of fibers to the areas of less thickness to a greater extent than to the areas of normal thickness by applying air pressure, and maintaining the difference in thickness until the fibers are set by continued application of air pressure.

3. The method of controlling the flow of fibers to form a paper sheet having designated areas of less thickness than the normal thickness of said sheet, which comprises restricting the flow of fibers to the areas of less thickness to a greater extent than to the areas of normal thickness by applying a confined current of air, and maintaining the difference in thickness until the fibers are set by continued application of said confined current of air.

4. The method of controlling the flow of fibers to form a paper sheet having designated areas of less thickness than the normal thickness of said sheet, which comprises

restricting the flow of fibers to the areas of less thickness to a greater extent than to the areas of normal thickness by applying air pressure over an area extending from the slice to a point at which the fibers are set.

5. The method of controlling the flow of fibers to form a paper sheet having designated areas of less thickness than the normal thickness of said sheet, which comprises restricting the flow of fibers to the areas of less thickness to a greater extent than to the areas of normal thickness by applying air pressures thereto.

10 In testimony whereof, I have signed my name to this specification this twelfth day of October, 1926.

RUPERT B. DANIELS.

20

25

30

35

40

45

50

55

60

65